

A. ISAACS,  
DUPLICATING ROLL OR SHEET AND PROCESS FOR MAKING SAME,  
APPLICATION FILED DEC. 15, 1914.

1,151,951.

Patented Aug. 31, 1915.

*Fig. 1*



*Fig. 2*



*Fig. 3*



WITNESSES

Geo. A. Senior

Edmond Livingstone Brown

INVENTOR:

Albert Isaacs

BY  
Edmond Congar Brown

ATTORNEY

# UNITED STATES PATENT OFFICE.

ALBERT ISAACS, OF NEW YORK, N. Y.

## DUPLICATING ROLL OR SHEET AND PROCESS FOR MAKING SAME.

1,151,951.

Specification of Letters Patent. Patented Aug. 31, 1915.

Application filed December 15, 1914. Serial No. 877,369.

*To all whom it may concern:*

Be it known that I, ALBERT ISAACS, a citizen of the United States, and a resident of the city and State of New York, have invented certain new and useful Improvements in Duplicating Rolls or Sheets and Processes for Making Same, of which the following is a specification.

My invention relates to duplicating rolls or sheets for duplicating machines, and to the processes by which same are made, and more particularly to an improved form of roll or sheet which will be lasting in quality and which cannot be easily torn, from which the coating is not easily removed, which will not dry out, and in which the fabric support of the gelatinous material will not leave an imprint on the said material or otherwise injure it when the sheet is rolled up.

The invention consists in the new and improved process by which such a roll or sheet is produced and in the sheet produced by said process, as illustrated by means of the accompanying drawings, and hereinafter more particularly described.

In the said drawings, Figure 1 is a cross-section of a portion of a duplicating roll or sheet constructed according to my invention in its simplest form; Fig. 2 is a similar cross-section of a modified form; and Fig. 3 is a perspective view of a portion of such a roll or sheet constructed according to my invention.

Heretofore, in order to produce duplicating rolls, a sheet or roll of oil-cloth has been covered on the raw side with several coats of linseed oil, and after allowing the same to dry thoroughly, a layer of hot gelatinous composition has been applied to the oil-coated side. It has been found, however, that the gelatinous composition dried out and becomes inelastic, rendering the sheet useless. In order to overcome this difficulty a different process has been used, consisting in coating the finished side of the oil-cloth with a layer of gelatinous composition. Rolls made by this process were less liable to dry out, but it was found that when the roll was rolled up the threads of the raw side of the cloth would imprint themselves upon the composition, destroying its smooth

surface. The present invention comprises a new process and new product eliminating the disadvantages above mentioned.

In carrying my invention into effect in the modification thereof, shown in Fig. 1, I provide a roll or sheet of fabric, adapted to form a support for the duplicating medium, said fabric being designated 11. One side of this fabric is coated with a suitable filler, which may be composed of, for instance, whiting, zinc, oxid, white lead, clays, or other suitable substances which when mixed with a drying oil, such as linseed oil, will serve to coat and fill in the said fabric, the materials used on this side of the fabric being preferably such as will be more or less adhesive to the gelatinous composition to be afterward applied. In the drawing this filler is designated 12. The other side of the fabric 11 is coated with a filler 14, which may be of a composition substantially similar to the filler 12, except that it is preferably made from such materials as are as far as possible non-adhesive to said gelatinous composition after the same has become set. One purpose of this filler is to prevent the weave of the fabric from impressing itself upon the duplicating surface, thus roughening the same and making it unfit for use. If desired, the surface of this filler 14 may be calendered so as to render the same smoother as well as more durable.

It is, of course, immaterial which of the two coatings above referred to is applied first, and they may be applied simultaneously if desired. After the fabric has been coated with the filler 12 it is covered on that side with a gelatinous duplicating composition 13, adapted to receive impressions made upon paper or the like with a suitable duplicating or copying ink, and to transfer such impressions to other sheets of paper or other suitable material. The gelatinous composition, heated to a suitable temperature, is applied so as to form a layer in contact with the filler 12, the heat temporarily softening the oil in the filler and causing the gelatinous composition to adhere.

In the form shown in Fig. 2, I also provide a fabric support, here designated 15, one side of which is coated with a filler 16, analogous to the filler 14 of Fig. 1, which

like the filler 14 may if desired be calen-  
dared. The other side of the fabric, which  
is to receive the gelatinous duplicating com-  
position is also coated with a filler 17, anal-  
ogous to the filler 12 of Fig. 1, although in  
this case it is not specially desirable that the  
filler be adhesive to said gelatinous compo-  
sition, as this filler 17 is coated with a layer  
18 of drying oil, or some similar substance,  
this layer causing the hot or liquid gelati-  
nous duplicating composition designated 19,  
to adhere to the filler 17 in a manner anal-  
ogous to that described above.

By the above process, a duplicating roll  
15 or sheet, may be produced in which the  
gelatine composition will not dry out, and  
in which the threads of the cloth will not  
imprint themselves upon the face of the  
gelatinous composition. It is not essential  
20 that the duplicating composition employed  
be a gelatinous composition, as a sheet com-  
prising any composition which may be ap-  
plied and which will adhere, and which will  
serve to receive and transfer impressions,  
25 will be within the spirit and scope of my  
invention.

Having thus described my invention what  
I claim as new and desire to secure by Let-  
ters Patent is as follows:

30 1. The process of producing a duplicating  
roll or sheet adapted to be rolled up upon  
itself which consists of coating a fabric with  
a filler on both sides, and coating one side of  
said fabric with a gelatinous duplicating  
35 composition.

2. The process of producing a duplicating  
roll or sheet adapted to be rolled up upon  
itself which consists of coating a fabric with  
a filler on both sides, one of said fillers being  
40 adhesive to a duplicating composition and  
coating said adhesive filler with a gelatinous  
duplicating composition.

3. The process of producing a duplicating  
roll or sheet adapted to be rolled up upon  
45 itself which consists of coating a fabric with  
a filler on both sides, one of said fillers being  
non-adhesive to a duplicating composition,  
and coating the side of said fabric not bear-  
ing the non-adhesive filler with a gelatinous  
50 duplicating composition.

4. The process of producing a duplicating  
roll or sheet adapted to be rolled up upon  
itself which consists of coating a fabric with  
a filler on both sides, coating one of said fill-  
55 ers with a substance adhesive to a duplicat-  
ing composition, and coating said adhesive  
substance with a duplicating gelatinous com-  
position.

5. The process of producing a duplicating  
60 roll or sheet adapted to be rolled up upon  
itself which consists of coating a fabric with  
a filler on both sides, one of said fillers being  
non-adhesive to a duplicating composition,  
coating the other of said fillers with a sub-  
65 stance adhesive to a duplicating composi-

tion, and coating said adhesive substance  
with a gelatinous duplicating composition.

6. The process of producing a duplicating  
roll or sheet adapted to be rolled up upon  
itself which consists of coating a fabric with  
70 a filler on both sides, one of said fillers being  
adhesive to a duplicating composition, and  
the other of said fillers being non-adhesive  
to a duplicating composition, calendering  
one of said fillers, and coating the other  
75 filler with a layer of gelatinous duplicating  
composition.

7. The process of producing a duplicating  
roll or sheet adapted to be rolled up upon  
itself which consists of coating a fabric with  
80 a filler on both sides, calendering one of said  
fillers, coating the other of said fillers with a  
substance adhesive to a duplicating composi-  
tion, and coating the said adhesive substance  
with a gelatinous duplicating composition.  
85

8. The process of producing a duplicating  
roll or sheet adapted to be rolled up upon  
itself which consists of coating a fabric with  
a filler on both sides, and coating one side of  
90 said fabric with a heated gelatinous dupli-  
cating composition.

9. A duplicating roll or sheet adapted to  
be rolled up upon itself comprising a fabric  
coated with a filler on both sides, and coated  
95 adhesive substance being coated with a ge-  
latinous duplicating composition.

10. A duplicating roll or sheet adapted to  
be rolled up upon itself comprising a fabric  
coated with a filler on both sides, one of said  
fillers being adhesive to a duplicating com-  
position, said adhesive filler being coated  
100 with a layer of a gelatinous duplicating com-  
position.

11. A duplicating roll or sheet adapted to  
be rolled up upon itself comprising a fabric  
coated with a filler on both sides, one of said  
fillers being non-adhesive to a duplicating  
105 composition, and the other filler being coated  
on one side with a layer of a gelatinous du-  
plicating composition.  
110

12. A duplicating roll or sheet adapted to  
be rolled up upon itself comprising a fabric  
coated with a filler on both sides, one of said  
fillers being coated with a substance ad-  
hesive to a duplicating composition and said  
115 adhesive substance being coated with a ge-  
latinous duplicating composition.

13. A duplicating roll or sheet adapted to  
be rolled up upon itself comprising a fabric  
coated with a filler on both sides, one of said  
fillers being non-adhesive to a duplicating  
120 composition, and the other filler coated with  
a substance adhesive to a duplicating com-  
position and said adhesive substance coated  
with a gelatinous duplicating composition.  
125

14. A duplicating roll or sheet adapted to  
be rolled up upon itself comprising a fabric  
coated with a filler on both sides, one of said  
fillers being adhesive to a duplicating com-  
position and coated with a layer of a ge-  
130

latinous duplicating composition, and the other filler being non-adhesive to a duplicating composition and calendered.

15. A duplicating roll or sheet adapted to be rolled up upon itself comprising a fabric coated with a filler on both sides, one of said fillers being coated with a substance adhesive to a duplicating composition and coated with a layer of gelatinous duplicating

composition, and the other filler being calen- 10 dered.

In witness whereof I have hereunto signed my name this 10th day of December 1914, in the presence of two subscribing witnesses.

ALBERT ISAACS.

Witnesses:

LOUISE ENDERLE,  
EDMOND CONGAR BROWN.

Correction in Letters Patent No. 1,151,951.

It is hereby certified that in Letters Patent No. 1,151,951, granted August 31, 1915, upon the application of Albert Isaacs, of New York, N. Y., for an improvement in "Duplicating Rolls or Sheets and Processes for Making Same," an error appears in the printed specification requiring correction as follows: Page 2, claim 9, strike out lines 95-96 and insert the words *on one side with a layer of gelatinous duplicating composition*; and that the said Letters Patent should be read with this correction therein that the same may conform to the record of the case in the Patent Office.

Signed and sealed this 18th day of January, A. D., 1916.

[SEAL.]

J. T. NEWTON,

*Acting Commissioner of Patents.*

Cl. 101—173.